

W. H. POWELL.

METHOD AND APPARATUS FOR MAKING PLATE GLASS.  
APPLICATION FILED DEC. 12, 1919.

1,381,591.

Patented June 14, 1921.

FIG. 1



FIG. 6



FIG. 2



FIG. 3



FIG. 4



FIG. 5



William H. Powell  
By Ray & Totten  
Atty.

# UNITED STATES PATENT OFFICE.

WILLIAM H. POWELL, OF ELMER, NEW JERSEY.

## METHOD AND APPARATUS FOR MAKING PLATE-GLASS.

1,381,591.

Specification of Letters Patent. Patented June 14, 1921.

Application filed December 12, 1919. Serial No. 344,365.

To all whom it may concern:

Be it known that I, WILLIAM H. POWELL, a citizen of the United States, and resident of Elmer, in the county of Salem and State 5 of New Jersey, have invented a new and useful Improvement in Methods and Apparatus for Making Plate-Glass; and I do hereby declare the following to be a full, clear, and exact description thereof.

10 My invention relates to the manufacture of plate glass and other articles formed from glass.

One object of my invention is to provide a method of making plate glass and the like 15 whereby the surfaces of the plate shall be given a smooth finish without grinding or other special polishing. Another object of my invention is to provide simple and effective apparatus for carrying out the above- 20 indicated method.

Generally stated, my method consists in casting a plate or other desired body of glass, allowing the glass to set with a smooth exposed surface, inverting the glass article 25 so produced upon a suitable support and then heating the rough upper surface of the inverted article while simultaneously applying a cooling medium to the smooth lower surface, with the result that the upper surface 30 is melted sufficiently to impart a perfectly smooth finish without melting the body of the article sufficiently to destroy the smoothness of the bottom surface.

In the accompanying drawing which 35 shows a simple form of apparatus for carrying out the above method, Figure 1 is a perspective view of a ladle or mold suitable for the casting operation; Fig. 2 is a longitudinal sectional view of the ladle shown in Fig. 40 1; Fig. 3 is a longitudinal central sectional view of a box-form adapted to support the glass plate in the reheating operation, the ladle being shown in inverted position over the box-form. Fig. 4 is a sectional view 45 similar to Fig. 3, but showing the plate in position on the box-form ready for reheating; Fig. 5 is a longitudinal sectional view showing somewhat diagrammatically a furnace with the box-form in position for the 50 further treatment of the plate; and Fig. 6 is a fragmentary vertical sectional view of a ladle or mold suitable for the production of beveled plate glass without grinding.

The ladle 1 shown in the drawing consists

of a base portion 2 of the size and shape to 55 be given the finished plate, and provided with a peripheral flange 3 and with a handle 4. While the ladle 1 is shown as rectangular in form, it may obviously be made circular or of any other desired shape, and 60 the base portion 2, instead of being flat, as shown, may be corrugated or provided with such other projections or depressions as are desired to appear in the finished plate.

The box-form shown in Figs. 3, 4 and 5 65 comprises a hollow body-portion 5 which may conveniently be formed of cast iron and which is provided around its upper surface 6 with a peripheral flange 7 similar to the flange 3 of the ladle 1. The space defined by 70 the flange 7 of the box-form should be of the same size and shape as the space contained in the ladle 1, in order that the glass plate A which is cast in the ladle may be properly received on the box-form. The upper surface 75 6 of the box-form is provided with a considerable number of perforations 8 and an inlet 9 is provided in one of the side walls of the box form and is connected through a valve 10 and a rubber hose or other flexible 80 connector 11 with a source of compressed air or other suitable cooling fluid.

In employing the above-described apparatus, the ladle 1 is filled with molten glass, preferably by dipping the ladle bodily into 85 a tank of melted glass, although the ladle may also be filled by pouring glass from the usual melting pot. The glass is allowed to remain in the ladle until it is set sufficiently 90 for handling and the glass adhering to the edges of the ladle may be trimmed off. If desired, the glass in the ladle may be smoothed by means of a suitable scraper or roller, but in that case care must be taken that the glass is sufficiently hot to restore its 95 smooth exposed surface. When the glass is sufficiently set, the ladle 1 is inverted over the box-form and the glass plate A is transferred to the perforated top of the box, the ladle being then removed. Heat is then applied to the upper surface of the plate, as it 100 rests upon the box-form, this being conveniently accomplished by moving the box-form bodily beneath a suitable furnace heated with gas or oil. Such a furnace is indicated, 105 somewhat diagrammatically, in Fig. 5, where the furnace casing 15 is shown as being provided with burners 16, an inspection window

17 and a sliding lower door 18 which may be pushed aside by the box-form and may be drawn forward to close the furnace when the box-form is removed. The particular heating means employed are not material to the present invention, and such means may take any convenient form. During the heating operation a cooling medium, preferably compressed air, is introduced into the interior of, 5 the box-form through the inlet 9 and is thereby directed against the under surface of the glass plate A through the openings 8. The heating is continued until the upper surface of the plate is seen to flow and assume a perfectly smooth condition, whereupon the box-form is removed from the furnace, or the heating is otherwise discontinued. The plate is allowed to cool and is found to be perfectly polished on both sides.

10 20 For the production of beveled plate glass according to my method, I employ a ladle or mold of the modified form shown in Fig. 6, having slanting flange portions 20 which impart the proper bevel to the plates 25 that are cast in the ladle. The beveled portions of the plate are polished along with the main body of the plate, as described above, and I am thus able to produce beveled glass without the usual grinding operation.

30 35 The above described method and apparatus are capable of numerous variations in accordance with the size and shape of the plates or other articles to be produced. In the production of large plates it will be desirable to provide the ladle 1 with trunnions or other suspension means in order to facilitate handling, and suitable arrangements for moving the box-forms and for discharging the finished plates may also be 40 employed.

45 Numerous variations may also be made in the construction of the box-form and in the particular manner in which the air, water or other cooling fluid is directed against the under side of the plate during the reheating operation. It is to be understood that my invention comprises all of these modifications, together with such other changes and adaptations as fall within the 50 scope of the appended claims.

What I claim is:

1. The method of making plate glass that comprises casting a plate of glass, inverting the cast plate, and heating the top of said inverted plate and thereby imparting a smooth surface thereto.

2. The method of making plate glass that comprises casting a plate of glass, inverting the cast plate, heating the top of the inverted plate to impart a smooth surface thereto, and simultaneously applying a cooling medium to the bottom of said inverted plate.

3. The method of making plate glass that comprises casting a plate of glass, inverting the cast plate upon a foraminous support,

bringing the said support beneath a source of heat and applying a cooling medium to the said plate from below through the openings in the said support.

4. The method of making plate glass that 70 comprises dipping molten glass in a ladle corresponding in size and shape to the finished plate, allowing the glass to set in the ladle, inverting the ladle to deposit the plate upon a foraminous support similar in 75 size and shape to said ladle, bringing the said support beneath a source of heat to impart a smooth upper surface to the inverted plate, and applying a cooling medium to said plate from below through the openings in the said support, to preserve the smooth lower surface of said plate.

5. The method of making plate glass that comprises dipping molten glass in a ladle corresponding in size and shape to the 85 finished plate, trimming the excess glass from the edges of said ladle, allowing the glass to set in said ladle, inverting the ladle to deposit the plate upon a foraminous support similar in size and shape to said ladle, 90 bringing said support beneath a source of heat to impart a smooth upper surface to the inverted plate, and applying cold air to said plate from below, through the openings in said support, to preserve the smooth 95 lower surface of said plate.

6. As a new article of manufacture, a plate of glass having a heat-polished beveled edge.

7. As a new article of manufacture, a 100 plate of glass having a beveled edge produced by casting and heat-polishing without grinding or pressing.

8. Glass-working apparatus comprising a foraminous support and a ladle or mold 105 of the same size and shape as the said support, and adapted to be inverted over the said support to transfer thereto a plate of glass or the like.

9. Glass-working apparatus comprising a 110 hollow metal box having an upstanding flange extending around one side thereof, the said side being provided with a plurality of perforations, means for introducing a cooling fluid into the interior of the said 115 box, and a ladle or mold of the same size and shape as the space defined by said flange, the said ladle or mold being adapted to be inverted over said support to transfer there-to a plate of glass or the like.

10. The method of making beveled plate glass that comprises placing molten glass in a ladle having beveled edges and corresponding in size and shape to the finished beveled plate, allowing the glass to set in said 125 ladle, removing the cast plate from said ladle, heating the beveled side of the said plate sufficiently to heat-polish its surface, and simultaneously cooling the original upper surface of said plate.

11. The method of making beveled plate glass that comprises placing molten glass in a ladle having beveled edges and corresponding in size and shape to the finished beveled plate, allowing the glass to set in said ladle, removing the cast plate from said ladle and inverting it upon a hollow support, placing said support beneath a source

of heat and simultaneously introducing a cooling medium into the said support. <sup>10</sup>

In testimony whereof I, the said WILLIAM H. POWELL, have hereunto set my hand.

WILLIAM H. POWELL.

Witness:

JOHN F. WILL.